# EUROPEAN PATENT APPLICATION

(11) **EP 0 332 698 A1**
(43) Date of publication of application: **20.09.1989**
(21) Application number: 87905651.3
(22) Date of filing: 27.08.1987
(51) Int. Cl.: C10M 107/34, C10N 40/04

(54) **GEAR OIL COMPOSITION**

(71) Applicant: Tonen Corporation, Tokyo (JP)
(72) Inventor: SUZUKI, Kuniaki, Tokyo 153 (JP)
(74) Representative: Holmes, Michael John
(86) International application number: JP8700636
(87) International publication number: WO8901964

(57) **Abstract**

A gear oil composition containing polyoxyalkylene glycol as a base oil, wherein the polyoxyalkylene glycol is a polymer obtained by ring-opening polymerization or ring-opening copolymerization of one or more members selected from among alkylene oxides having 2 to 4 carbon atoms and having a viscosity of 5 mm²/s to less than 20 mm²/s (at 100°C). This gear composition has remarkably excellent oxidation stability and abrasion resistance at elevated temperatures and a good flowability at low temperatures.

ABSTRACT

A gear oil composition comprising polyoxyalkylene glycol(s) as a base oil, characterized in that said polyoxyalkylene glycol(s) are polymer(s) obtained by ring-opening polymerization or copolymerization of one or more alkylene oxides selected from the group of alkylene oxides having 2 to 4 carbon atoms and have a viscosity of 5 mm²/s to 20 mm²/s at 100°C.

This gear oil composition exhibits excellent properties in oxidation stability and wear resistance at high temperatures as well as in flowability at low temperatures.

## Description

### FIELD OF THE INVENTION

This invention relates to a gear oil composition comprising polyoxyalkylene glycol(s) (also called simply polyglycol(s)) in this specification as a base oil. More particularly, it relates to a gear oil composition whose wear resistance and oxidation stability are improved by incorporating polyoxyalkylene glycol(s) having specific viscosity properties as a base oil.

### BACKGROUND OF THE INVENTION

Mechanical devices using gears have been utilized in a variety of industrial fields because they steadily transmit power to a driven device. Depending on their usage these gear devices are broadly classified into industrial devices and those for use in automobiles. An appropriate gear oil suitable for the particular purpose is employed in each case.

A gear oil is a lubricant oil which reduces friction between at least one pair of gears transmitting power from a driving device, e.g., a motor, to a driven one, thereby decreasing power loss and inhibiting damage to the gears, thus prolonging the life span of the gears. Presently mineral oils are exclusively employed as base oils of gear oils. Gear oils further contain approximately 0.1 to 10 % by weight of various additives such as antioxidants, extreme pressure agents, rust preventives and anti- foaming agents.

Recently machines made in Japan have been exported to various countries, including the U.S.A. and European countries, and shipments thereof have been increasing yearly. It is now a usual practice to supply lubricants, e.g., gear oils, to such exported machines in the manufacturing plant prior to their shipment. Therefore it is necessary to take into consideration the properties of these lubricants in light of the working conditions in the customer country. Thus the machine manufacturers have requested the lubricant oil manufacturers to supply products possessing properties that meet the trends of the demand (the market circumstances). In compliance with the wishes of the former, the latter have attempted to develop products satisfying these requirements.

In Japan, base oils comprising mineral oils are mainly employed in gear oils. When it is required to use gears at, for example, high temperatures or high loads, a gear oil composition comprising such a base oil, as well as specific additives such as extreme-pressure agents or antioxidants, is usually employed.

An example of these gear oils is a lubricant oil composition disclosed in Japanese Patent Laid-Open No. 59-75995, wherein it is proposed to improve the wear resistance, extreme-pressure qualities, and friction properties of a lubricant oil by introducing an organo molybdenum compound of a specific structural formula and an acid phosphite ester or an acid phosphate ester as essential ingredients into, for example, a mineral oil having a lubricant viscosity. These gear oils comprising mineral oils as base oils have been exclusively used in Japan, since mineral oils are relatively inexpensive; and a base oil for a gear oil use in conventional gear devices may be obtained by removing impurities such as unsaturated hydrocarbons and metallic components from a raw mineral oil through solvent-refining or hydrogenation.

There have been attempts to use synthetic lubricant oils comprising, for example, esters, poly-α-olefins and polyglycol oils. Generally, a synthetic lubricant oil of the desired lubricant properties may be obtained by controlling the synthesis conditions. Thus it is believed that synthetic lubricant oils can exhibit better anti-friction and anti-oxidation properties than mineral oils. As for polyglycol oils, Japanese Patent Publication No. 49-1339 has disclosed a lubricant which is prepared by adding, for example, an aromatic amine, an aliphatic phenol and an organic phosphate to a base oil. This lubricant composition has improved oxidation stability, load resistance and rust resistance at high working temperatures.

Recently the property requirements of gear oils, particularly the wear resistance and oxidation stability at high working temperatures, have become more stringent. Presently, gear oils comprising mineral oils as base oils have an overwhelming share in the field of machine industries. However, gear oils which comprise a mineral base oil containing additives compensating for the shortcomings of the mineral base oil will not satisfy the various requirements of future markets. Thus it is impossible to provide gear oils possessing excellent properties unless the properties of mineral oils, which are contained therein in an amount of 70 to 95 % as base oils, are improved.

Under these circumstances it is necessary to reconsider the use of synthetic lubricant oils as base oils of gear oils. However there is presently no commercially available synthetic lubricant oil which has the requisite satisfactory properties and is also inexpensive. Regarding polyglycol oil, the relationship between its properties as a base oil and its molecular structure is not yet fully understood. Thus, efforts in this area have been directed to identifying suitable types and amounts of additives for conventional base oils. In addition, a polyglycol gear oil is liable to exhibit poor cold viscosity properties when used in a machine in a cold environment, resulting in failure during normal operation of the transmission device.

### DISCLOSURE OF THE INVENTION

It is an object of the present invention to provide a low cost gear oil comprising a synthetic lubricant oil which, without requiring additives, has high wear resistance, excellent stability at high temperatures and high- or moderate-speed rotation, and high flowability at low temperatures.

Under these circumstances, we have attempted to overcome the above problems and consequently found that a gear oil comprising specific polyoxyalkylene glycol(s) as a base oil exhibits not only a remarkably improved wear resistance and oxidation stability, even at high temperatures, but also improved viscosity properties at low temperatures.

Accordingly, the present invention resides in a gear oil composition comprising polyoxyalkylene glycol(s) as a base oil wherein said polyoxyalkylene glycol(s) are polymer(s) obtained by ring-opening (co-) polymerization of one or more alkylene oxides selected from the group of alkylene oxides having two to four carbon atoms and have a viscosity of 5 mm²/s to 20 mm²/s at 100°C.

We first describe the polyoxyalkylene glycol(s) of the present invention. The polyglycol(s) of the present invention are polymer(s) obtained by ring-opening (co-)polymerization of one or more alkylene oxides selected from the group of alkylene oxides having two to four carbon atoms, i.e., ethylene oxides, propylene oxides, butylene oxides and isobutylene oxides. Therefore the polyglycols include, for example, polyethylene glycol, polypropylene glycol, polybutylene glycol, polyisobutylene glycol, a ring-opened copolymer of ethylene oxide and propylene oxide, and a ring-opened copolymer of propylene oxide and butylene oxide. The average molecular weight of these polyalkylene glycols is approximately 800 to 2300. For example, polypropylene glycol of an average molecular weight of 1000 to 2000 may be employed in the present invention. It is required that such a polyoxyalkylene glycol have specific viscosity properties. Namely, the viscosity thereof at 100°C should be from 5 mm²/s to 20 mm²/s. A polyoxyalkylene glycol having a viscosity lower than 5 mm²/s at 100°C is undesirable because of its poor wear resistance and low oxidation stability at high temperatures. On the other hand, one having a viscosity higher than 20 mm²/S is also undesirable because its poor flowability at low temperatures will result in insufficient lubricating effects. A gear oil that is to be used in a machine in a cold area is particularly required to have satisfactory viscosities at low temperatures. It is possible to achieve a good lubricating effect by employing in the present invention polyoxyalkylene glycol(s) having a viscosity of 6 x 10⁴ mPa.s to 95 x 10⁴ mPa.s at -40°C. A particularly preferred base oil for the gear oil of the present invention comprises polypropylene glycol or polyethylene glycol having a viscosity of 8 mm²/s to 19.8 mm²/s at 100°C and 10 x 10⁴ mPa.s to 40 x 10⁴ mPa.s at -40°C.

The polyoxyalkylene glycol(s) of the present invention can be produced by known methods. For example, polypropylene glycol can be obtained by polymerizing propylene oxide in the presence of a metal alcoholate as a catalyst and water or an alcohol as a initiator under a pressure of 1 to 10 atm at 100 to 150°C.

As the polyoxyalkylene glycol(s) of the present invention polypropylene glycol may be used alone. Alternately a base oil which is a mixture of polypropylene glycol and polyethylene glycol or polybutylene glycol may be used. It is highly effective to use a base oil comprising such a mixture of polyoxyalkylene glycols for achieving the viscosity properties as described above. That is to say, a polyoxyalkylene glycol base oil having appropriate viscosity properties can be readily obtained by blending polypropylene glycol, which has a high molecular weight and a high viscosity at low temperatures, with polyethylene glycol, which has a relatively low molecular weight and is highly flowable at low temperatures. Similarly the polyoxyalkylene glycol(s) of the present invention may be blended with esters. Examples of these esters are monoesters, diesters and polyesters, i.e., those having three or more ester bonds. The monoesters include aliphatic esters having 15 or more carbon atoms; the diesters include those formed by esterifying aliphatic dibasic acids having 4 to 14 carbon atoms with monoalcohols having 4 to 14 carbon atoms; and the polyesters include triesters formed from trihydric alcohols having 4 to 13 carbon atoms and fatty acids having 3 to 13 carbon atoms and tetraesters formed from tetra-hydric alcohols having 5 to 10 carbon atoms and fatty acids having 5 to 10 carbon atoms. Among these esters diesters such as diisodecyl adipate, dioctyl sebacate and dioctyl azelate, and triesters such as trimethylolpropane triheptanoate and trimethylolpropane trioctanoate are particularly preferred. These esters enhance the oxidation stability of polyalkylene glycols. In particular, the addition of approximately 10 to 50 % by weight of the ester(s) can significantly enhance the lubricant properties of a gear oil comprising polyalkylene glycol(s) of a low viscosity, i.e., 5 to 20 mm²/s at 100°C, as a base oil.

The polyglycol synthetic lubricant oil of the present invention can be used as a gear oil. It exhibits remarkable effects, particularly when used as an industrial gear oil. Namely, it is useful as a gear oil utilized at high temperatures and high load or under unsettled temperature conditions, i.e., widely varying from low temperatures to high temperatures. The polyglycol base oil may further contain conventional additives, depending on its application. Suitable additives include antioxidants such as aromatic amines (0.3 to 5 % by weight); extreme pressure agents such as tricresyl phosphate (0.3 to 13 % by weight); metal inactivators (0.01 to 3 % by weight); rust preventives (0.05 to 2 % by weight); oiliness improvers (0.01 to 3 % by weight); and anti-foaming agents (0.0005 to 0.02 % by weight). These additives may be added in a total amount of 3 to 15 % by weight and, unlike a mineral base oil, no viscosity index additive is required.

Since the polyoxyalkylene glycols are polyether(s) wherein oxyalkylene(s) are polymerized through a ring-opening mechanism, the polyoxyalkylene glycol(s) of the present invention have high oxidation stability and flowability even at high temperatures. Furthermore, they can act as a viscosity index improver since they have specific viscosities at both high and low temperatures. Although the presence of the hydroxyl (alcohol) groups at the ends of the polyoxyalkylene glycol(s) may decrease the oxidation stability thereof at high temperatures, the lubricant properties of the gear oil product are not affected thereby since the base oil shows excellent interaction with antioxidants such as aromatic amine compounds.

### THE OPTIMUM EMBODIMENTS OF THE INVENTION

### EXAMPLES 1 - 6

Gear oil compositions (A to F) of the present invention were prepared by using a polyoxyalkylene glycol (polypropylene glycol or polyethylene glycol) as a base oil and adding tricresyl phosphate as an extreme-pressure agent and an aromatic amine antioxidant thereto. Table 1 shows the composition of each gear oil thus obtained and the viscosity properties thereof at 100°C and -40°C.

The wear resistance of each gear oil composition of the present invention thus prepared was determined in the following manner: a four-ball wear tester (Shell type) was operated at an oil temperature of 150°C, at a rate of 1800 rpm under a load of 25 kg for 30 minutes, and then the wear diameter of a roller (1/2 inch) was determined. Table 2 shows the results.

Then an IEA gear tester was operated at an oil temperature of 140°C at a gear rate of 7000 rpm under a load of 60 lbs for three hours. Subsequently the weight loss in large and small gears was determined. Table 2 shows the results.

Further, the oxidation stability of each gear oil composition of the present invention was also determined according to Fed. 791 b. 5308 at an oil temperature of 150°C for 200 hours. The change in viscosity (% @ 100°C), the total acid number gain (mg KOH/g), insoluble matters in oil (% by weight; determined by the pentane-B method) and the change in the weight of metals, i.e., iron and copper (mg/cm²), were determined. Table 2 shows the results.

### COMPARATIVE EXAMPLES 1-4

Comparative gear oils (a to d) were prepared by adding appropriate amounts of various additives such as a viscosity index improver, an antiwear agent and an antioxidant to commercially available base oils which were ATF-D II, ATF-D II′, Gear oil 75W-90 and a diester oil (DIDA; diisodecyl adipate), although no viscosity index improver was added to the diester oil. Table 1 shows the composition and properties of each gear oil thus obtained.

These comparative gear oils were subjected to the same procedures as those described in Examples 1 to 6 to determine the wear resistances and oxidation stabilities thereof. Table 2 shows the lubricant properties.

The above Examples 1 to 6 and Comparative Examples 1 to 4 indicate that the polyglycol gear oils of the present invention have almost the same wear resistances as those of the conventional ATF-D II and Gear Oil 75W-90 but are superior to these conventional oils in viscosity properties and oxidation stabilities. It was also found that the polyglycol gear oils of the present invention had remarkably improved wear resistances and viscosity properties compared with the diester oil (DIDA).

**Table 1**

| Gear oil composition | | | | | | | | | |
|---|---|---|---|---|---|---|---|---|---|
| | Base Oil | | | | Additive (% by wt.) | Viscosity | | | |
| | Glycol | | Mineral Oil | Diester | | 100°C (*mm*²/s) | | -40°C (mPa·s) | |
| | PPG | PEG | | | | Base oil | Product | Base oil | Product |
| A | 90 | | | | 10 | 8.50 | 8.25 | 11×10⁴ | 16×10⁴ |
| B | 90 | | | | 10 | 9.50 | 9.15 | 14×10⁴ | 20×10⁴ |
| C | 90 | | | | 10 | 17.0 | 15.7 | 28×10⁴ | 40×10⁴ |
| D | 90 | | | | 10 | 19.8 | 18.1 | 39×10⁴ | 56×10⁴ |
| E | | 90 | | | 10 | 9.00 | 9.10 | - | - |
| F | | 90 | | | 10 | 16.5 | 14.8 | - | - |
| a | | | 85 | | 15 | 4.0 | 7.21 | solidified | 4.2×10⁴ |
| b | | | 85 | | 15 | 4.5 | 8.50 | do. | 10×10⁴ |
| c | | | 70 | | 30 | 4.0 | 14.20 | do. | 14.8×10⁴ |
| d | | | | 90 | 10 | 3.68 | 3.80 | 0.345×10⁴ | 0.48×10⁴ |

| Note: | | | | | | | | | |
|---|---|---|---|---|---|---|---|---|---|
| *: A to F and d contain tricresyl phosphate and an aromatic amine but no viscosity index improver. | | | | | | | | | |
| a and b contain 7 % by weight of a viscosity index improver. | | | | | | | | | |
| c contains 20 % by weight of a viscosity index improver. | | | | | | | | | |

**Table 2**

| Properties | | | | | | | | | | |
|---|---|---|---|---|---|---|---|---|---|---|
| | Example | | | | | | Comparison | | | |
| | 1 | 2 | 3 | 4 | 5 | 6 | 1 | 2 | 3 | 4 |
| | A | B | C | D | E | F | a | b | c | d |
| | PPG | | | | PEG | | ATF-DII | ATF-DII′ | 75W90 | DIDA |
| Viscosity property | ○ | ○ | ○ | ○ | ○ | ○ | × | × | × | Δ |
| 4-ball wear test wear diameter (*mm*) | 0.45 | 0.35 | 0.31 | 0.30 | 0.37 | 0.33 | 0.48 | 0.46 | 0.42 | 0.50 |
| 1AE gear test gear wt. loss (*mg*) | 110 | 65 | 18 | 10 | 70 | 20 | 80 | 75 | 34 | 200 |
| Change in viscosity (%) @ 100°C | 1.00 | 1.00 | 1.02 | 1.01 | 1.03 | 1.03 | 1.06 | 1.06 | 1.12 | 1.01 |
| Total acid number gain (*mg*KOH / *g*) | 0.8 | 0.7 | 0.4 | 0.4 | 0.75 | 0.4 | 1.50 | 1.40 | 2.50 | 0.10 |
| Insoluble materials in oil (wt. %) | 0.03 | 0.03 | 0.01 | 0.01 | 0.02 | 0.02 | 0.05 | 0.05 | 3.40 | 0.01 |

| Change in metal weight | | | | | | | | | | |
|---|---|---|---|---|---|---|---|---|---|---|
| Fe (*mg*/*cm*²) | -0.02 | -0.02 | -0.01 | +0.01 | ±0.01 | ±0.00 | -0.03 | +0.01 | -0.03 | +0.01 |
| Cu (*mg*/*cm*²) | +0.01 | +0.01 | ±0.00 | -0.01 | -0.10 | -0.10 | -1.40 | -1.35 | -61.2 | -0.01 |

### INDUSTRIAL AVAILABILITY

The polyoxyalkylene glycol synthetic lubricant oils of the present invention, which exhibit a high oxidation stability and wear resistance at high temperatures and high flowability at low temperatures, undergo less denaturation than conventional mineral oil- or ester-based lubricant oils. Thus, they can be used at a low cost with little or no maintenance.

## Claims

A gear oil composition comprising polyoxyalkylene glycol(s) as a base oil, characterized in that said polyoxyalkylene glycol(s) are polymer(s) obtained by ring-opening polymerization or copolymerization of one or more alkylene oxides selected from the group of alkylene oxides having 2 to 4 carbon atoms and have a viscosity of 5 mm²/s to 20 mm²/s at 100°C.
